

No. 806,045.

PATENTED NOV. 28, 1905.

R. BAGGALEY & C. M. ALLEN.

METHOD OF CONVERTING MATTE.

APPLICATION FILED JULY 18, 1904. RENEWED APR. 6, 1905.

3 SHEETS—SHEET 1.

Fig. 2.



Fig. 1.



WITNESSES

*L. A. Comer*  
*Franklin T. Lang*

INVENTORS

Ralph Baggaley  
Charles M. Allen  
by Bancroft & Byrnes  
their Attorneys

No. 806,045.

PATENTED NOV. 28, 1905.

R. BAGGLEY & C. M. ALLEN.  
METHOD OF CONVERTING MATTE.

APPLICATION FILED JULY 18, 1904. RENEWED APR. 6, 1905.

3 SHEETS—SHEET 2.

Fig. 2.



Fig. 3.



WITNESSES

*L. A. Conroy*  
*Frank M. Clancy*

INVENTORS

Ralph Baggley  
Charles M. Allen  
by Bancroft & Byrnes  
their Attorneys

No. 806,045.

PATENTED NOV. 28, 1905.

R. BAGGALLEY & C. M. ALLEN.

METHOD OF CONVERTING MATTE.

APPLICATION FILED JULY 18, 1904. RENEWED APR. 6, 1905.

3 SHEETS—SHEET 3.

Fig. 6.



Fig. 5.



WITNESSES

L. H. Conroy  
Frank M. Ceburg

INVENTORS

Ralph Baggaley  
Charles M. Allen  
by Bassett & Barnes  
their attorneys

# UNITED STATES PATENT OFFICE.

RALPH BAGGALEY, OF PITTSBURG, PENNSYLVANIA, AND CHARLES M. ALLEN, OF LOLO, MONTANA; SAID ALLEN ASSIGNOR TO SAID BAGGALEY.

## METHOD OF CONVERTING MATTE.

No. 806,045.

Specification of Letters Patent.

Patented Nov. 28, 1905.

Application filed July 18, 1904. Renewed April 6, 1905. Serial No. 254,112.

*To all whom it may concern:*

Be it known that we, RALPH BAGGALEY, of the city of Pittsburgh, in the county of Allegheny and State of Pennsylvania, and CHARLES M. ALLEN, of Lolo, in the county of Missoula and State of Montana, have invented a new and useful Method of Converting Matte, of which the following is a full, clear, and exact description, reference being had to the accompanying drawings, forming part of this specification, in which—

Figure 1 shows a longitudinal central section of an ore-lined converter suitable for practicing our invention. Fig. 2 is a vertical cross-section on the line II II of Fig. 1. Fig. 3 is a vertical longitudinal section of a converter suitable for the practice of a modification of our invention wherein the ores are attached to the converter by partial fusion. Fig. 4 is a vertical cross-section on the line IV IV of Fig. 3. Fig. 5 is a vertical longitudinal section of a water-jacketed converter for practicing a modification of our invention. Fig. 6 is a vertical cross-section on the lines VI VI of Fig. 5.

The object of our invention is to reduce the cost of producing blister-copper by eliminating the present heavy expenses for converter-linings and to transform this serious expense into a source of profit, thus constituting a new method of converting mattes.

In the practice of our invention three things are of importance: first, that the converter-walls should be either composed of heavy metal blocks of such relative thickness that they cannot be destroyed during the process or preferably of heavy metal blocks with a light basic interior lining, which will also resist injurious action by the oxidized iron, such as must always result where silica is used in direct contact with matte that contains iron and also to the end that the converter-walls may be comparatively clean and hot after the layer of ore has been consumed and dissolved by the action of the matte and heat; second, that the converter shall be so designed and made of such materials that it may be able to withstand without injury the great heat of the process as well as the intensely corrosive action of the fiery low-grade matte; third, that the converter may be able to withstand this exacting service without unduly abstracting and dissipating the internal heat that is gen-

erated by and that is essential to the success of the process.

The apparatus which we prefer to use in practicing our invention is composed of heavy metal blocks, whose thickness bears a proper relative proportion to the molten bath to be held, as fully explained in application, Serial No. 200,943, filed March 31, 1904, and which is lined, preferably, with magnesite brick, as shown in Figs. 3 and 4. Another good form of apparatus is that shown in Figs. 1 and 2.

The water-jacketed converter shown in Figs. 5 and 6 can be used in practicing this art; but we recommend that at the later stages of the process the flow of water through the jackets be greatly reduced or preferably shut off altogether for a time in order to prevent any excessive abstraction of heat from the vessel.

Many efforts have been made in the past to utilize mineral-bearing ores as the source of silica for fluxing the iron of copper matte after the latter has been oxidized by the converting-blast. As a rule these efforts have taken the form of the use of pulverized ores mixed with clay or some other bonding agent and water into a plastic mass with which the converter is lined.

In John Holway's Patent No. 234,129, dated November 9, 1880, a process is described wherein silicious and slag-producing materials are added to the matte. Metalliferous substances containing the necessary slag-producing materials and containing also valuable metals in such small quantities as to make them unfit for treatment by themselves are described as preferable.

In actual work John Holway reported to the London Society of Arts that he used quartz-sand impregnated with about five per cent. of oxid of iron. He fed this with a shovel into the converter's mouth, but without success.

Attempts have been made to supply silica or silicious ore in pulverized form by injecting it with the blast into the molten bath; but this process has not been successful.

It has also been proposed to utilize ores that contained not less than eighty-five per cent. of silica and whose distinctive feature was silver values, and to each ton of pulverized argentiferous quartz to add one hundred and seventy-five pounds of fire-clay, with suitable

proportions of water to make a plastic lining for the converter to flux the oxidized iron of the molten bath. This process has also remained to the present day unused.

5 At Aguas Calientes a very unusual ore obtained from the St. Gertrude mine, in Pachuca, Mexico, has been utilized as a successful converter-lining and fluxing agent. This ore contains approximately eighty per cent. of 10 pure quartz, twenty per cent. of almost pure alumina, and from eight dollars to fifteen dollars per ton in gold values, which latter are finely and evenly disseminated through the quartz. The ore is pulverized in Chilean 15 mills, is then mixed with suitable proportions of water, and in this form it is rammed as a lining into very large converter-shells, usually to a thickness of about twenty-four inches.

It has also been proposed, though without 20 success, to feed white-hot silica into the mouth of the converter.

In the process described in a patent of 25 Ralph Baggaley, No. 746,241, dated December 8, 1903, cold silica in solid form was fed into the converter either on top of a clean body of molten converter-matte or preferably 30 into an empty heated converter, where it was agglutinated by auxiliary heat, and thereafter the body of molten converter-matte was poured into the converter upon it.

Ralph Baggaley's Patent No. 746,260, dated December 8, 1903, described a like process to that described in No. 746,241, except that it utilized mineral-bearing silicious ores as the 35 fluxing material.

In all former efforts to use ore for converter-linings or to utilize either ore or silica by introducing it through the twyers or into the mouth of the converter the aim has been 40 to satisfy the iron in a high-grade converter-matte and by this means to increase the percentage of the mineral contents, which would also have the effect of decreasing the volume of the molten bath correspondingly through 45 the separation of slag. All such attempts to use ores for lining have been very costly, because such ores must be first pulverized, which in itself is very expensive, then thoroughly mixed with water, and with one exception 50 with clay, and thereafter they must be tamped or compacted into the converter-shell with rammers in order that they would remain firmly in position during the converting process. It has been found that the best results 55 are obtained if only a moderate quantity of water be used; but in order to secure such comparatively dry plastic mixture in its position in the converter-shell a large amount of hand-labor has been required in the work of 60 ramming it. This process has also required the expenditure of money for coke with which to dry out the linings before use, and inasmuch as coke is always expensive in localities where copper ores are treated this has 65 added materially to the cost. In actual prac-

tice it is found that only a small proportion of such lining can be used until the destructive action must cease, else the destruction of the metal converter-shell will quickly follow, inasmuch as the corrosive action of the bases 70 is not and cannot be distributed evenly over the surface of the acid lining. On the contrary, the iron of the matte attacks the silica of the lining much more at some places than it does at others. Hence when it has weakened it at any one point to the extent that the metal shell becomes heated to a red heat further converting action must cease or serious and permanent injury to the shell will result. When a lining thus becomes weakened, it necessitates the removal of a large amount of the same in order to prepare the shell for relining, and the portion removed usually is 80 so permeated with fusible material from the former charges that it is unfit to be used 85 again for a lining material. It must be smelted as a means of recovering its contained values, which process involves additional expense. It is estimated that each converter-lining costs at least forty dollars. If carefully prepared, it may last for from seven to 90 twelve blows; but if carelessly applied it may be destroyed in a single blow or in two or three blows. Under the most favorable circumstances a very large proportion of the 95 material contained in each lining is useless for effective work, because the iron of the matte usually eats holes through certain portions of it, thus rendering the balance useless for fluxing purposes. The life of such a lining 100 will be very largely governed by the care and the uniform ramming exercised by the workmen while placing it in position. The constant aim has been to make the lining as durable as possible as a measure of economy. 105 This has led experimenters to avoid everything that would render the lining friable or easily dissolved by the molten bath, and it has therefore been considered necessary to avoid the use of all ores and all lining materials that carry basic elements or compounds, 110 inasmuch as these would contribute to its rapid destruction. Every other consideration has been sacrificed in the effort to maintain the life of the lining to the utmost. By 115 our invention this practice is entirely reversed, and inasmuch as we depend upon the destruction of the lining material as the means whereby we extract and recover mineral values contained in the ores of which we make 120 the lining economy demands that the destruction be rapid, since in this way a greatly-increased amount of effective work can be accomplished in a given time.

Our present invention affords the first 125 method that is adapted to the use of a lining containing ores carrying sulfids of the base metals in combination with silica.

For the reasons above stated all past experimenters have been forced to compound 130

their lining material with alumina or some equivalent bonding agent mixed with water, and where ores were used at all as lining material only such were used as contained high 5 percentages of silica and such as contained no metals other than gold or silver, (preferably in a finely-disseminated state.) Ores which contained base metals—sulfids, arsenids, antimonids, or any of the elements or compounds 10 usually found in ores—or such as would readily be dissolved, and indeed all ores which contained matte-making elements or compounds were avoided.

In present practice, where mattes are low 15 grade in copper values—say below forty per cent., inasmuch as practically the entire remaining sixty per cent., constituting a much larger proportion of the total bulk of the charge, must be removed in the converting 20 process—it has been found necessary either to add additional matte in the molten state from time to time or else to combine charges of matte by transferring partially-blown charges from one converter into another as 25 a means of securing sufficient material with which to finish a charge to blister-copper.

In the Bingham Cañon district in Utah many vast bodies of low-grade sulfid ores are found ordinarily containing mineral values 30 varying from four dollars and fifty cents to five dollars and eighty cents per ton. The proportion of copper amounts to one or 1.5 per cent., and the remaining values consist usually of gold and to a small extent of silver. In a single instance ores of this character contained total values of seventeen dollars per ton, the copper varying from one to two per cent. and the remaining values consisting principally of gold and silver. These 35 ores at present are smelted in the ordinary water-jacketed blast-furnace with coke and with slow smelting as a means of enriching them as much as possible before converting. The resulting matte after the first fusion in 40 the blast-furnace, containing from eight to ten per cent. of mineral values, is transferred to a number of silica-lined converters, and it causes a rapid destruction of their linings, owing to the heavy percentage of iron. A 45 large proportion of worthless slag is produced, and the proportion of resultant concentrated matte is consequently extremely small. In order to conduct this tedious process on commercial lines, it has been found 50 necessary to transfer these small amounts of concentrated matte from a number of different converters into one in order to produce one full molten bath of, say, forty to fifty per cent. converter matte, and after consolidating 55 many such charges they are thereafter brought up to the grade of blister-copper in a single silica-lined converter.

By our present invention we depart widely 60 from prior practice, because we utilize as a fluxing agent ores that carry varying per-

centages of bases, sulfids, and basic compounds. We thus establish the conditions necessary to furnish a constantly-increasing supply of matte of general composition, and we gradually and constantly add percentages 70 of mineral values to our matte, so that we are enabled either to finish the process, or, if desired, to bring up the grade of our matte to forty or fifty per cent. of copper, or to even a higher grade, if such is desired. This produces what is commonly called “converter-matte” without resorting to any of the present wasteful and expensive processes of concentration by water or by fire. In prior processes ores have with the one exception here- 80 in referred to been unfit for use as lining for the reason they all contain percentages of basic elements or compounds and are hence unfit for lining converters on the lines of present practice. The reason that an ore 85 lining for converters has been successful at Aguas Calientes, in Mexico, the one exception above referred to, is because the very unusual ore there used is practically free from all basic elements or compounds excepting alumina. In our present invention we can successfully use ores carrying large percentages of bases and basic sulfids, and the presence of these hitherto-objectionable elements and compounds will materially contribute to 90 the speed and to the success of the process and will augment the mineral values contained in the bath. We are enabled to add copper, iron, sulfids, gold, silver, and any matte-making elements or compounds by means of our 95 lining, and any and all copper, gold, and silver thus contributed to the bath through the medium of our lining will add to the enrichment of our matte.

Our present invention in intent and effect 105 is the reverse of all prior efforts to convert mattes, as it offers the only instance wherein it is possible to operate economically with a converter wherein the lining material is entirely consumed in one converting operation 110 and also wherein the converter itself is thereafter in a suitable condition to admit of continuous work without additional expense for renewals or for repairs.

In the metallurgy of copper a greater necessity exists for exact weights and exact proportions than perhaps in any other science. It is of the first importance that the proportions, for instance, of silica, lime, iron, sulfur, &c., should be exact by weight and that 115 guesswork should not be relied on for these things. It is useless to predetermine proportions by assay if such proportions are not subsequently delivered. If they be not delivered, exact work is impossible.

Our present invention affords the only instance in the metallurgy of copper where one can calculate in advance the exact amount of acid or of base that will be dissolved and that will be actually received into the molten bath 120 125 130

to produce expected results, inasmuch as we dissolve it all. In all past processes the quantity or proportion of silica that is dissolved from the converter-lining must necessarily be 5 an unknown quantity, for no one can tell in advance how much or how little of it will be dissolved. For this reason our present invention affords a scientific method where actual figures based on the chemical equivalents of 10 the elements contained in the ore or silica lining can be arrived at.

In the practice of our invention we preferably take a converter—such, for example, as shown in Figs. 1 and 2, which is made of 15 thick metal blocks 2 and which may be provided with a magnesite-brick interior lining—and apply to its interior a body or coating of copper ores containing silica and containing also sulfids of iron, copper, &c., and preferably gold, silver, and matte-making elements or compounds. We prefer to apply 20 this lining by distributing on the interior of the converter a coating of slag or matte in a liquid condition and then to apply the ore lining 25 to the coated interior and to cause it to adhere thereto, after which it may, if desired, be cemented with another addition of slag or matte. The converter being in a heated condition, we run into it from a smelting-furnace, 30 forehearth, or other convenient source a body of molten slag, preferably enough to equal in volume one-half the usual converter charge, or we may use for this purpose some molten matte. We then tip the converter back and 35 forth on its axis, so as to distribute this slag or matte over the interior surface in a sticky layer *b*, as shown in Figs. 1 and 2, and we then tip the converter completely to discharge the surplus. The body of ore is then added 40 to the converter, and by rocking the latter back and forth it is tumbled over the layer *b* and caused to adhere thereto in a layer *c*, or, if desired, the ore may be spread over the converter with a shovel or otherwise. A 45 small quantity of molten matte or slag is then preferably poured into the converter and being distributed in like manner over the ore or silica lining completes the bonding of the particles. The slag or matte quickly sets, 50 and, if desired, this setting can be hastened by blowing air thereon from the twyers 3. The ore is thus held to the converter with sufficient security to serve as a lining and to supply the flux to the charge beneath the 55 bath; but being open and unpacked the lining acts more readily and causes the converting operation to proceed more quickly than is possible with linings heretofore employed.

Instead of first distributing a layer of molten 60 matte or slag over the converter before applying the lining material we may place such material in the converter and cause it to adhere thereto by pouring upon it a small volume of molten slag or matte.

65 The lining may be constituted by selecting

such ores as contain a sufficient quantity of flux, such as oxids or sulfids, to enable the lining to be cintered in place by the application of external heat from oil-burners or the like.

70 Instead of using a converter made of metal blocks, as shown in Figs. 1 and 2, we may employ the converter shown in Figs. 5 and 6, having an exterior water-jacket 4 and an interior lining 5 of magnesite, within which the lining *c* of ore is applied. We may also use apparatus such as shown in Figs. 3 and 4, in which the converter-shell is constituted of heavy metal blocks 2, having an interior lining 5 of magnesite brick, within which the ore lining *c* is placed, as above described. We also show in this converter burners for supplying flame by which the ore lining may be cintered in place. These burners may be omitted when the ore body is cemented to the 85 interior walls by molten matte or slag.

The quantity of ore employed as lining material is selected with reference to the composition of the matte to be treated. It should contain sufficient silica to flux all the ore contained in the matte that is delivered into the converter as well as the additions thereto supplied by the fusing of the matte-making compounds introduced with the ore. The amount of ore is preferably so determined 90 that the entire mass will be consumed in a single blow of the converter. It will be patent to those who are conversant with the art of converting that every substance added to the charge as slag-making material will absorb and will carry away with it an appreciable amount of copper, and that the more foreign material that is introduced into the slag the greater will be the loss of copper. It then follows that any additions of silicious or 100 aluminous substances will aggravate such copper losses, in exact proportion to the amount of such additions.

There is no known way, either by fire, by 110 water, or by leaching, commercially speaking, whereby the silica contained in sulfid ores can be removed from the ore without a corresponding loss of the sulfids themselves. Therefore any method that enables the operator to use the same kind of ore for the 115 converter-lining that is used to produce the matte to be converted must effect an important saving in all of the values that would be stolen by substances used for lining that are derived from other sources than the matte-making ore itself.

120 While in the foregoing description we have specifically described converter-walls composed of heavy metal blocks, of heavy metal blocks supplemented with an interior basic 125 lining and water-jacketed walls supplemented with an interior basic lining, we do not limit our invention thereto, but intend in our broader claims to claim our new method when practiced with apparatus of any kind. Thus 130

within the scope of our broader claims the ore lining above described may be applied to a converter having a compact silica lining providing the ore lining contains approximately sufficient flux to satisfy the body of

5 matte, after the latter has been supplemented by the additions resulting from the melting of the ore lining itself. When such is used, the bath will attack the loose ore lining so 10 much more rapidly than it can attack the compact silica lining, that successful practice of our invention can be attained.

15 Doubtless many variations in this process will suggest themselves to those skilled in the art; but,

20 Having devised the only method that has ever been used that is adapted to utilize the same kind of ore for lining the converters that is smelted to produce the matte for the converter, we claim—

25 1. The method herein described of converting matte, which consists in subjecting matte to an air-blast in a converter having an uncompacted lining, composed of the same material as the ore to produce the matte to be converted; substantially as described.

30 2. The method herein described of converting matte, which consists in introducing a body of matte into a converter lined with a body of value-bearing ore loosely held together, and subjecting the matte to an air-blast; substantially as described.

35 3. The method herein described of converting matte, which consists in introducing a body of matte into a converter lined with a body of value-bearing ore loosely held together without aluminous bonding material, and subjecting the matte to an air-blast; substantially as described.

40 4. The method herein described of converting matte, which consists in introducing matte into a converter having a lining containing silica and sulfids of the base metals, as a means of increasing the volume of the matte and 45 fluxing the same, and subjecting the matte to an air-blast; substantially as described.

5. The method herein described of converting matte, which consists in applying to a

converter a lining of ore containing matte-making material, introducing matte thereinto, 50 and subjecting the same to an air-blast; substantially as described.

6. The method herein described of converting matte, which consists in applying to a converter a lining of ore containing silica and 55 matte-making material; adding thereto a body of low-grade matte; fluxing the iron of such matte with the silica of the ore and augmenting its volume with the matte-making material; substantially as described.

60 7. The method herein described of converting matte, which consists in applying to a converter a lining of ore; supplying matte thereto; blowing air thereinto and consuming the entire body of the lining in the converting 65 operation; substantially as described.

8. The method herein described of converting matte, which consists in applying to a converter a lining containing ore in a pre-determined amount; supplying matte thereto; 70 blowing air thereinto and consuming the entire body of the lining in the converting operation; substantially as described.

9. The method herein described of converting matte, which consists in applying to a non-silicious converter-wall, a loose body containing matte-making compounds and silica and introducing low-grade matte thereto, and subjecting the same to an air-blast; substantially 75 as described.

80 10. The method herein described of converting matte, which consists in applying to a non-silicious converter-wall, a loose lining containing matte-making compounds and silica, in amount sufficient to flux the compounds 85 of the matte to be fluxed; introducing low-grade matte thereto and consuming said lining in a single converting operation; substantially as described.

85 In testimony whereof we have hereunto set 90 our hands.

RALPH BAGGALY.  
CHARLES M. ALLEN.

Witnesses:

WILLIAM M. KIRKPATRICK,  
FRANK L. RILEY.